

BEST AVAILABLE COPY

W. E. SHERBONDY.

PROCESS FOR FORMING A SHEET METAL SHELL FOR A SPARK PLUG.

APPLICATION FILED AUG. 7, 1914.

1,152,983.

Patented Sept. 7, 1915.

2 SHEETS—SHEET 1.



WITNESSES:

Spud Klotzbach  
J. Bresel

Fig. 14.



BY

William E. Sherbondy  
by John W. Mooney  
ATTORNEY

INVENTOR.

W. E. SHERBONDY.

PROCESS FOR FORMING A SHEET METAL SHELL FOR A SPARK PLUG.

APPLICATION FILED AUG. 7, 1914.

1,152,983.

Patented Sept. 7, 1915.

2 SHEETS-SHEET 2.



WITNESSES:

Frank Klotzbach Fig. 14  
R. B. Reed I

INVENTOR.

William E. Sherbondy  
by Wm. E. Sherbondy  
ATTORNEYS.

# UNITED STATES PATENT OFFICE.

WILLIAM E. SHERBONDY, OF CLEVELAND, OHIO, ASSIGNOR, BY MESNE ASSIGNMENTS,  
TO THE BIGSBY ROTARY MANUFACTURING COMPANY, OF CLEVELAND, OHIO, A  
CORPORATION OF OHIO.

## PROCESS FOR FORMING A SHEET-METAL SHELL FOR A SPARK-PLUG.

1,152,983.

Specification of Letters Patent. Patented Sept. 7, 1915.

Application filed August 7, 1914. Serial No. 855,601.

*To all whom it may concern:*

Be it known that I, WILLIAM E. SHERBONDY, a citizen of the United States, and resident of Cleveland, in the county of Cuyahoga and State of Ohio, have invented certain new and useful Improvements in Process for Forming a Sheet-Metal Shell for a Spark-Plug, of which I hereby declare the following to be a full, clear, and exact 10 description, such as will enable others skilled in the art to which it appertains to make and use the same.

The objects of the invention are to provide a mechanical process comprising step 15 by step operations whereby the shell of a metal spark plug can be constructed from sheet metal, and provided with an opening for the accommodation of the electrode.

At the present time a large expense has 20 to be incurred in the installment of automatically acting machinery to construct the spark plugs from bar metal stock, which necessitates a large amount of waste in scrapped material, and although in every 25 way an inefficient and expensive method of producing the plugs it has hitherto been an unavoidable one, since no other method has been known.

By means of the present improved process 30 the shells can be produced from sheet metal by means of drawing and forming dies and parts which have hitherto been difficult of shaping on account of the hexagonal sides and angles and inner and outer 35 shoulders can be manufactured at a much greater rate of speed and with comparatively little loss of material in the form of scrap.

The amount of labor involved in producing 40 the shells and the accompanying expense is also very greatly reduced. Further, the initial expense of the sheet metal employed in the manufacture of shells for spark plugs is reduced from 50% to 65% below the expense 45 of manufacturing the shells from bar stock, and substantially also without any waste of material in forming the body of the plug, after the blank has been cut.

Further, important features comprise the 50 completion of the shell from a sheet metal blank into the conformation desired with the fewest number of operations compatible with the perfect shaping thereof.

The difficulties encountered are greatly increased by the peculiar shape of the shell, 55 the extreme thickness of the sheet metal required, and the small diameter of the parts to be formed.

To accomplish the desired results particular attention has been paid to the features 60 required in the several dies to obtain the greatest efficiency in each step of the process without which it would be impossible to carry out the various succeeding steps.

The several steps of the process and the 65 manner of obtaining the gradual changes in the shape of the sheet metal to produce the finished article are illustrated in the accompanying drawings, hereinafter described, and clearly pointed out in the 70 claims.

In the accompanying drawings Figure 1 is a vertical central section showing the sheet metal blank from which the body of the shell of a spark plug is formed and the 75 dies for cutting out the same; Fig. 2 is a similar section showing the blank formed into the shape of a cup and the forming dies therefor, and also a stripping device; Fig. 3 is a similar section showing the 80 method of further elongating the cup, reducing the diameter of the lower portion thereof while retaining the diameter and somewhat upsetting the upper portion of the shell; Fig. 4 is a section similar to Fig. 85 3, showing the same function carried further and the lower portion of the cup still further reduced in diameter, and elongated, preparatory to forming the hexagonal faces upon the upper portion of the cup; Fig. 5 90 is a similar section showing the same functions for the dies that are shown in Figs. 3 and 4, and forming the body of the shell ready for the hexagonal shape of the upper portion; Fig. 6 is a similar section showing 95 the first step in the method of expanding and shaping the hexagonal exterior surfaces of the enlarged portion of the body; Fig. 7 is a plan view of the die; Fig. 8 is a sectional view showing a continuation of the 100 process of reducing the hexagonal portion in diameter and elongating it; Fig. 9 is a plan view thereof; Fig. 10 is a similar view showing the hexagonal portion still further reduced and elongated; Fig. 11 is a plan 105 view thereof; Fig. 12 is a similar section

showing the final formation, including upsetting the body portion and giving the precise finished shape and size to every part; Fig. 13 is a similar view showing the cutting away of the end of the shell of the spark plug to provide an opening through which the inner electrode may project; Fig. 14 is a side elevation of a finished shell showing a metal washer sleeved thereover to provide the necessary shoulder.

There are several sizes and varieties of shells for spark plugs in general use of which the two most common have respectively straight parallel sides and tapered sides upon their inner extremities, both are screw threaded for attachment to the cylinders of explosion engines. The shell having straight parallel sides is provided with an annular projecting shoulder or a metal ring seated upon shoulders at the angles takes the place of the projecting shoulder to make the plug gas tight. The shell having tapered sides does not require this shoulder since it closes the opening completely. Both shells are provided with hexagonal sides at their upper extremities and both can be made by this process.

As stated very heavy material is required in the construction of the spark plugs for the purposes of first obtaining the exterior shape and for cutting the screw thread therein and secondly to enable the internal shoulder to be formed, which is the seat of the inner insulation or core; and to cut a screw thread if desired within the body wall to retain the bushing or sleeve nut that ordinarily secures the insulation in place.

In order to produce a hollow body or shell having an exterior portion shaped in the form of an accurate hexagon of given dimensions it is absolutely necessary to make the cup shown in Fig. 2 of a definite fixed outside diameter, to give a definite diameter across the flat portions of the hexagon, and this diameter must be retained throughout all the operations, up to the forming of the angles, and if it is not retained it is impossible to get a perfect hexagon.

Many other features are found to be of the greatest importance. For instance it has been found that the disk shaped blank must accurately fit the recess made for it in the die or the top edge of the cup will be very uneven and after a few operations of the dies the amount of unevenness would multiply to such an extent that the piece could not be used.

The exact diameter of the first blank requires careful experiment and calculation and is not an obvious thing to the best skilled mechanics, since many features which are learned only by experiment control the subsequent shaping of the metal.

The radius marked  $\alpha$  in Fig. 2 must be

of an exact predetermined length or when the blank is formed the metal will stretch and form an imperfect end. When however this radius is exactly right and the dies are of the right size the tendency of the metal is to thicken out the upper portion of the cup, which is of a very important feature, so as to provide substance sufficient to fill out the angles of the hexagon later on in the process, but which must be gradually provided for during the process.

Many experimental forms of dies ineffectually employed to produce the hexagonal body, and the cups have been formed of various sizes and the lower portions have been reduced and elongated and the cup has been then drawn through a hexagonal die, but after carrying out the remaining steps of the process the hexagonal portion has not been properly filled out, nor has the proper thickness of material been retained for the seat of the insulation or for the inside screw thread which receives the screw threaded clamping sleeve. Afterward a split die of hexagonal shape was attempted, the two halves of which were driven together, and produced a clamping effect upon a large portion of the shell, but after many attempts had been made to employ this die it was given up as equally impractical as the previous trials. Afterward a cup having a reduced lower portion was driven through a die having hexagonal sides, the male die or punch fitting the lower portion of the shell and the upper portion hexagonal, and made to exactly fit the hexagonal die, but the results were unsatisfactory. Finally a punch and die were formed as shown in Fig. 3 with better results but not yet perfect. It was found that only by making a combination punch having a sleeve thereon, the lower portion of which engages the upper portion of the shell so as to retain the shell when the lower portion of the cup is being reduced in diameter and elongated, the upper portion will be retained of the proper size and will be somewhat upset, which will produce the required thickness for the hexagonal part, the shoulder and the inner thread.

The various steps of the process until the shell of the spark plug is completed and the various tools employed and the peculiarities of their construction may be described as follows: In Fig. 1 a sheet of metal  $M$  is placed upon a female die  $A$  and a male die  $B$  of the same diameter is employed to strike out the disk shaped blank  $C$  from which the shell of the spark plug is formed. In Fig. 2 the next step of the process is illustrated where the disk  $C$  is shown resting in a recess  $C'$ , of precisely the same diameter as the disk so as to accurately center it and which is formed in a block  $C^2$ . The block  $C^2$  is provided with the cylindrical opening

$C^3$  which is expanded at  $A$  at the upper end so as to enter the recess  $C'$  in a smooth gradual curve. The blank is forced through this opening by means of a punch  $D$  having a 5 rounded lower end which forms the cup. The important feature of this step of the process is found in the action of the rounded corners  $A$  of this die, the radius of which is such as to permit the sides of the cup to 10 be elongated without cracking, which would be the result if the shoulder were abrupt.

In Fig. 3 the next step of the process is shown. Here  $E$  is a punch which has a reduced diameter  $E'$  which enters the cup as it 15 lies over the cylindrical opening  $F$  in the die block  $F'$ . This opening is of less diameter than the cup. The upper corners of this opening are rounded at  $F^2$  to permit drawing the cup to a reduced size and forming 20 the shoulder  $F^3$  thereon. As soon as the punch enters the cup and commences drawing the same down into the die, a sleeve  $G$  comes into play and forces the cup downward, in unison with the drawing movement 25 of the punch, until the lower extremity of the shell has been sufficiently elongated. The sleeve  $G$  will then compress the upper edge of the shell until it is slightly upset and at the same time the precise internal diameter 30 of the upper end of the cup is retained by the main body of the punch  $F$ . A shoulder  $F^3$  on the punch between the portions of different diameter forms the shoulder upon the inner surface of the shell, and an annular rib 35  $G'$  upon the lower extremity of the sleeve controls the external diameter thereof.

In Fig. 4 forming dies of similar shape are employed but the lower extremity of the punch and die are reduced in diameter to 40 still further elongate the cup and reduce the diameter of the lower end, so as to be nearly ready for the screw threading of the outer side of the shell. The shoulder formed upon the shell is made with a curve of increased 45 radius as the lower portion is reduced in size, the utility of which is hereafter explained.

It has been found necessary that the punch and die shall be in absolute alinement with 50 each other, so that the punch will be perfectly concentric with the die when it enters it, otherwise the upper and lower portions of the shell would not be in perfect alinement, or concentric with each other, and if any eccentricity should occur when the hexagonal portion is formed, it would have one side much longer than another, after the shell has been put through the subsequent operations of the process. To produce a perfect 55 hexagon a special gage has been made for alining these tools. The exact amount of upsetting of the upper end must also be carefully calculated to obtain the precise amount of material required to fill out the angles of 60 the hexagon upon that end. If necessary a

third operation with the punch and sleeve can be carried out to reduce the cup and to obtain the more perfect form as shown in Fig. 5. After the portions of two diameters described are thus formed it is usually necessary to anneal the cup to remove its hardness before the final operations of producing the hexagon upon the upper half thereof is carried out.

In Fig. 5 the radius from which the shoulder is formed upon the shell is still greater in length to obtain a larger curve therein, and is obtained by the reduction in size of the lower end of the cup while the size of the upper end of the cup remains unchanged.

The method of forming the hexagon is illustrated in Figs. 6, 7 and 8 respectively.

In Fig. 6 a punch  $H$  is formed of two diameters to correspond more closely to the finished diameters of the shell, the upper portion being of less diameter than the internal diameter of the upper portion of the shell as it leaves the dies shown in Fig. 5, but is larger than the finished diameter of the inside of the upper part of the shell. I 90 is the female die which forms the exterior of the hexagon. It will be seen that the opening in this die is approximately hexagonal in shape but the corners are extended outwardly or radially at  $I^2$  and the upper edges of the sides and corners are curved outwardly at  $I^2$  to permit the metal to flow gradually into the corners so as to fill out the hexagonal shape.

All the dies shown in Figs. 6, 7, and 8 are provided with rounded corners at  $I^2$  but the radial extensions of these corners are gradually reduced until only sharp hexagonal corners remain, and in the last used die the final shape is produced. As many intermediate dies may be used as are necessary to draw down the sides into a hexagonal form.

It has been found impracticable to produce hexagonal sides and perfectly sharp angles upon a cylindrical shell by means of dies of perfect hexagonal shape and having perfect angles, for the reason that a prohibitive number of operations would be required, hence the modifications heretofore described have been made.

The curves provided at the upper edges at  $J^2$ ,  $J^2$ , must be carefully considered in order to enable the larger portion of the shell to enter the die as easily as possible, and this curve should be a compound curve or cycloidal in shape, and extended low into the die, in a graceful curve, otherwise the reduced extremity of the punch will force a hole in the bottom of the cup before the larger portion of the shell can be drawn down through the die, expressed outward to fill the angles of the hexagon. Also the shoulder upon the shell should not be too abrupt or the effect would be the same, to cause the punch to force out the bottom of

the shell before the resistance of the thickened and enlarged portion of the shell has been overcome.

As shown in Fig. 6 the upper portion of the shell is of less diameter than the extreme diameter of the lip of the die at  $J^2$ , and hence the shell will partially enter the die before the drawing action commences and will be easily started down the curved edges of the die and centered therein. The gentle slope of the die and the large curvature of the shoulder on the shell coact to overcome the great resistance of the large portion of the shell to the drawing action of the punch. The fact that the shell is wholly within the curved portion of the die when that action commences also facilitates the result. In Fig. 12 a punch  $L$  having a shoulder  $L'$  operates in connection with the die  $N$  to compress the cup into perfect final shape.

In Fig. 13 dies are shown which cut the opening in the cup shaped extremity of the shell and comprise the punch  $P$  and female die  $P'$  which cut a portion from the extremity of the cup.

In Fig. 14 a ring or metal washer  $W$  is employed to obtain the necessary shoulder to form a gas tight joint when a straight parallel sided shell is used. A slight taper at  $W'$  insures a tight joint. The angles in this case are turned away to make a sharp corner against which the ring fits closely.

Having described the invention what I claim as new and desire to secure by Letters Patent is:

1. An improved method of producing a sheet metal shell for a spark plug, consisting in first cutting a disk of predetermined size from sheet metal from which all the integral parts are to be formed, second, drawing the disk laterally into a cupped form, while retaining it accurately in absolutely concentric dies, third, further reducing the lower portion while retaining the diameter of the upper portion substantially constant, said diameter of the upper portion being proportionately greater than the outer dimensions of the finished hexagon, next still further reducing the diameter of the lower portion while retaining the diameter of the upper portion substantially unchanged, next drawing the cup shaped blank having the reduced and elongated lower extremity through a forming die for the upper extremity, and thereby forming hexagonal sides, and radially and outwardly extending corners thereon, gradually reducing and elongating the sides and reducing the corners, and finally compressing and upsetting the upper portion until the perfect shape is attained.

2. The improved method of constructing a spark plug having a hexagonal upper portion and a reduced lower extremity from sheet metal, consisting in first, cutting a cir-

cular blank of predetermined size, second, drawing the same laterally into a cup form of predetermined larger diameter than the finished hexagon, drawing out the lower portion, while retaining the diameter of the upper portion substantially unchanged, and thickening slightly the wall of the upper portion to provide material for the angles of the hexagon, continuing the reduction of the lower portion and slightly elongating the same while retaining the diameter of the upper portion constant and finally forcing the shell through a die having a hexagonal opening of less diameter than the diameter of the upper portion of said shell, to form the hexagonal sides thereon.

3. An improved method of producing the shell of a spark plug from sheet metal having an opening in the lower end to receive the electrode, said shell having a hexagonal upper portion and a reduced lower portion consisting in first cutting a blank disk of predetermined diameter, drawing the same internally into cup form of greater diameter than the greater diameter of the finished shell, then drawing out the lower end of the cup to elongate it and reduce it in diameter while retaining the diameter of the upper portion unchanged and simultaneously slightly thickening the wall of the upper portion, repeating this operation until the lower portion is of the prescribed diameter and thickness, reducing the diameter of the upper portion of the cup and simultaneously forming hexagonal sides thereon, and finally cutting away a portion of the lower extremity of the cup to form an opening therethrough.

4. An improved process for constructing a shell for a spark plug from sheet metal, having an opening in the lower end to allow for electrode, consisting in, first cutting a blank in the form of a flat disk from sheet metal, supporting the same in a closely fitting die, and drawing the disk laterally by means of an accurately concentric punch to form a cup having its upper edges in a common horizontal plane gradually drawing out the lower portion to reduce its diameter and elongate the same, and simultaneously forming a shoulder thereon, and retaining the diameter of the upper portion substantially unchanged, and slightly upsetting the upper portion to thicken the metal therein, continuing this part of the operation until the lower part is substantially of the required diameter, then annealing the shell, and afterward forcing it through a hexagonal die of less diameter than the larger diameter of the cup.

5. An improved process for constructing a shell for a spark plug, having an opening in the lower end to allow for an electrode, consisting in first cutting a circular blank of predetermined size from sheet metal, draw-

- ing out the disk laterally to form a cup, drawing out the lower portion of the cup to elongate it and reduce it in size, and meanwhile retaining the upper portion of the cup 5 in a fixed position, and slightly upsetting the same to provide for the increased amount of metal required in filling out the corners of the hexagon, further reducing the diameter of the lower portion and elongat- 10 ing the same until the approximate shape of the lower portion has been secured, and meanwhile rigidly holding the upper portion and slightly upsetting the same, annealing the cup, drawing the cup through a 15 hexagonal die of less diameter than the cup, and of approximately the finished size of the shell, to form sides upon the upper portion of the cup and to elongate the same, giving a final pressure to the cup in dies or 20 finished sizes, and removing a portion of the lower end of the cup to form an opening for the passage of the electrode.
6. An improved method of forming a shell for a spark plug from sheet metal, having 25 an opening in the lower end to allow for electrode, consisting in first forming a cup from a sheet metal blank, reducing the diameter of the lower end thereof and elongating the same, the diameter of the upper portion remaining unchanged and larger than the diameter of the finished hexagon, slightly thickening the upper portion drawing out the upper end of the cup to form 30 hexagonal sides thereon and radially ex- 35 tended angles and continuing the procedure by redrawing the cup to gradually reduce and elongate the hexagonal portion, and re- 40 duce the projections at the angles until the required shape and size has been approxi- 45 mately attained, and finally compressing the shell within closed dies, to further elongate the lower portion, and accurately form the upper portion to give final shape desired.
7. The method of forming a cup shaped form having a reduced and elongated lower 50 extremity from which form a shell for a spark plug can be made, consisting in first cutting a disk of predetermined diameter from sheet metal, drawing the same into 55 cupped form, and retaining the edges in a common plane, supporting the cup upon a die of less diameter than the cup and having rounded edges, drawing the lower portion while retaining the diameter of the upper portion by means of a punch of true di- 60 ameter, the upper diameter preventing the reduction of the upper portion and exerting a pressure upon the upper portion in a lon- 65 gitudinal or axial direction to upset the same after the punch has entered the lower portion, so as to provide material from which the angles of the hexagon can be subse- 70 quently formed, and shoulder for the insula- 75 tion to rest upon, and in the inner face of which the screw thread can be cut.
- In testimony whereof, I hereunto set my hand this 24th day of July 1914.
- WILLIAM E. SHERBONDY.

In presence of—  
RALPH W. JEREMIAH,  
WM. M. MONROE.